

Jan. 23, 1934.

A. P. ROUX

1,944,759

DRAWING DIE

Original Filed Sept. 12, 1929

*Fig. 1.*



*Fig. 2.*



*Fig. 3.*



INVENTOR

Adrian P. Roux

BY

Emery, Booth, Verner & Whittier

ATTORNEYS

## UNITED STATES PATENT OFFICE

1,944,759

## DRAWING DIE

Adrian P. Roux, Oriskany, N. Y., assignor to  
 General Cable Corporation, New York, N. Y., a  
 corporation of New Jersey

Original application September 12, 1929, Serial  
 No. 391,994. Divided and this application July  
 8, 1930. Serial No. 466,442

8 Claims. (Cl. 205—29)

This invention relates to drawing dies and has  
 for an object the provision of an improved die.  
 This application is a division of my application,  
 Serial Number 391,994, filed September 12th,  
 5 1929.

Although there is a constant search for sub-  
 stitutes for diamond dies, up to the present time  
 none has been found which possesses all the de-  
 sirable qualities of diamond. But diamonds are  
 10 very expensive especially in larger sizes and are  
 difficult to mount satisfactorily. They are also  
 brittle and have other undesired characteristics.  
 As will be disclosed hereinbelow I have provided  
 a mounting for diamonds or other hard die cores  
 15 which permits the use of very small sizes, and  
 which furnishes so substantial a backing or ma-  
 trix for them that their tendency to split is  
 greatly reduced and they can be used until only  
 a thin shell or ring remains.

20 It has been the practice to some extent to  
 cast a body or matrix of iron, steel, bronze or  
 other metal upon the diamond or other hard ob-  
 ject as a core and then to pierce the blank thus  
 formed through the hard core to form the die.

25 But the matrix materials heretofore used or pro-  
 posed have not proven satisfactory. They are  
 not sufficiently hard or are too ductile or too elas-  
 tic to properly take the strains transmitted  
 30 through the core; or they do not closely overlie  
 and conform to the core due to improper shrink-  
 age or non-affinity for the core-piece. According-  
 ing to the present invention a suitable matrix  
 material and a proper process of surrounding  
 35 the core piece therewith have been discovered

so that the resultant die is adequately backed,  
 the matrix material being sufficiently hard, in-  
 elastic, non-ductile and non-brittle so that it will  
 not readily split or permit the core piece to split  
 40 and so closely and evenly overlying the core  
 piece that no inequality of strain is permitted.  
 Indeed, in the case where a diamond core is used  
 the matrix material is found to be so closely  
 adherent to the core as apparently to form a  
 45 union therewith.

50 The nature and objects of the invention will  
 be better understood from an exposition of an  
 exemplary and illustrative embodiment thereof  
 when considered in connection with the accom-  
 panying drawing, wherein:

Fig. 1 is a cross-section of a die and holder,  
 the view being taken on the line 1—1 of Fig. 2;

Fig. 2 is a plan view thereof; and

Fig. 3 is a section through a mold assembly  
 with the die in process of formation therein.

55 As shown in the drawing a hard core 10, for

example, a diamond, is encased in a matrix 11  
 of the desired material. These elements form-  
 ing the die proper are closely fitted into a hold-  
 er 12 and if desired may be driven or welded  
 therein. The assembly thus formed is in con-  
 dition for mounting in a drawing machine so  
 as to have wire or the like drawn therethrough  
 in the direction of the arrow A in Fig. 1.

The matrix material at present preferred may  
 have the following composition:

|                  | Per cent |
|------------------|----------|
| Iron             | 10       |
| Nickel           | 15       |
| Tungsten         | 30       |
| Tungsten carbide | 45       |
|                  | 70       |

But either iron or nickel may be used alone with  
 the tungsten carbide, or the tungsten may be  
 omitted, or the ratios of the various constituents  
 may be varied. In some cases cobalt may be  
 75 substituted for the iron or nickel or tungsten or  
 all of them. In any case the composition formed  
 will be extremely hard and tough and will have  
 good die-forming qualities of itself.

The die may be formed in a welding-carbon  
 mold 15 disposed between water-cooled electrodes  
 E1 and E2. The matrix material is preferably  
 finely divided (say 300 mesh) tungsten carbide  
 and metal which have been thoroughly mixed.  
 The diamond or other core piece is held centered  
 80 by projections 16 formed on the ends of carbon  
 plugs 17 which also confine the matrix material  
 about the core piece.

When thus assembled a considerable resilient  
 pressure (say 1100 pounds per square inch) is  
 imposed upon the carbon plugs 17 and electric  
 current is turned on the electrodes. This sinters  
 85 the matrix material and causes it to shrink in  
 volume, the projections 16 of the carbon plugs  
 17 burning away or breaking down sufficiently  
 to allow the plugs to follow up and maintain  
 pressure upon the matrix material.

After sintering the pressure is left on the plugs  
 while the die blank is allowed to cool between  
 the water-cooled electrodes. It is an inherent  
 fact that the matrix composed of these constitu-  
 ents and formed in this manner will be substan-  
 tially free from voids, which is to say, that the  
 voids, which are incident to sintering without  
 pressure are so markedly reduced as to make  
 it proper to say that the material is substantially  
 90 free from voids.

Upon cooling, the die blank thus produced  
 is pierced through the core piece with the re-  
 stricted portion of the pierced bore where the

110

greatest drawing strains will be imposed located in the hard core piece. Normally the indentations in the blank left by the plug projections 16 serve to locate the line of piercing. The blank 5 is then mounted in the holder 12 ready to be placed on a machine.

After the bore has become worn by use it may be re-bored for larger sizes and this may be repeated until the core is practically all used up 10 to a thin outer shell. This benefit is attained in part because of the superior matrix material provided which is so hard and otherwise suitable that it may itself well serve for the flaring portions of the drawing bore.

15 Furthermore, with such a matrix, much smaller diamonds or other hard cores may be successfully used initially than with any known settings. For example, where  $\frac{1}{4}$  carat diamonds were formerly used for steel settings, and 1 carat diamonds for bronze settings,  $\frac{1}{8}$  carat diamonds can by the present invention be used with equally good results; and likewise where  $1\frac{1}{2}$  carat diamonds were required for steel settings and 4 carat diamonds for bronze settings,  $\frac{3}{4}$  carat 20 diamonds can now be used. The saving, it will be realized, will be much greater than is represented by the proportions in size because of the fact that diamonds and other gems are disproportionately cheaper in the smaller sizes.

25 30 Also the cost of manufacture is greatly reduced by the present process. By comparison, in a large shop it has been found that sixty (60) of the new die settings can be made in the time that was formerly required to make ten (10) by 35 the old processes and materials. But above this is the fact that the dies made according to the present invention are practically all found by test to be free of faults while cast-metal set dies previously made were subject to many flaws and 40 faults, most of which could not be readily detected. So that, not only the settings, but the much more valuable cores were frequently broken before they had given much service in the expected way.

45 In service the setting material is unaffected by high temperatures which formerly rendered

useless dies having settings of other materials such as steel, bronze, etc.

The above description of the particular embodiment of the invention is illustrative merely and is not intended as defining the limits of the 80 invention.

What I claim is:

1. A drawing die comprising a diamond core embedded in a matrix formed of a tungsten carbide composition which is substantially free from voids, the die being pierced through the core to form the drawing bore and the restricted portion of the bore being located in the core. 85

2. A drawing die comprising a hard natural gem core embedded in a matrix formed of a tungsten carbide composition which is substantially free from voids, the die being pierced through the core to form the drawing bore and the restricted portion of the bore being located in the core. 90

3. A drawing die comprising a hard natural gem core embedded in a matrix formed of a composition including tungsten carbide and a metal of the iron group. 95

4. A drawing die comprising a hard natural gem core embedded in a matrix formed of a composition including tungsten carbide and a metal. 100

5. A drawing die comprising a hard natural gem core embedded in a matrix formed of a composition having approximately the composition, 105 iron 10%, nickel 15%, tungsten 30%, and tungsten carbide 45%.

6. A drawing die comprising a hard natural gem core embedded in a matrix formed of material including tungsten carbide. 110

7. A drawing die comprising a diamond core embedded in a matrix including a hard metal carbide which closely conforms to all contours of the core and intimately contacts with the same. 115

8. A drawing die comprising a diamond core 115 and an enveloping matrix of a composition which includes tungsten carbide, the matrix closely conforming to all contours of the core and intimately contacting the same.

ADRIAN P. ROUX. 120

50

125

55

130

60

135

65

140

70

145

75

150